

Nov. 15, 1927.

J. A. GANN

1,649,521

MAGNESIUM ALLOY

Filed Oct. 27, 1921



INVENTOR.

John A. Gann  
BY  
Day, Oberlin & Day  
ATTORNEYS

## UNITED STATES PATENT OFFICE.

JOHN A. GANN, OF MIDLAND, MICHIGAN, ASSIGNOR TO THE DOW CHEMICAL COMPANY, OF MIDLAND, MICHIGAN, A CORPORATION OF MICHIGAN.

## MAGNESIUM ALLOY.

Application filed October 27, 1921. Serial No. 510,796.

The present improved alloy is one in which magnesium is the predominant element, the object being to develop an alloy that will possess the characteristic lightness 5 which is obtained by the use of magnesium in excess of 80 per cent, while such alloy will be characterized by high tensile strength and hardness, coupled with moderate brittleness, as well as have a high melting point 10 and high thermal conductivity.

The field of use in the mechanical arts to which an alloy possessing the lightness and physical characteristics enumerated above 15 may be applied is extensive and need not be described in detail for the purpose in hand. Where it is desired to increase the hardness and/or at the same time reduce the brittleness of the alloy, the character of the latter may be modified by adding one or more 20 other metals in varying quantities, as will be hereinafter explained, the present invention consisting of an alloy of magnesium and nickel with or without the addition of such further metals together with the steps 25 involved in the making of such alloy herein-after fully described and particularly pointed out in the claims. The annexed drawing and the following description it will be understood set forth several of the various 30 ways in which the principle of the invention may be carried out.

In said annexed drawing:—

The single figure there appearing is a diagrammatic representation of certain physical 35 properties discovered in a binary magnesium-nickel alloy of the class in hand.

In said diagrammatic drawing the physical properties represented, it will be noted, are the impact-toughness, hardness and tensile strength of the alloy, the hardness being determined by the Brinell method and scaled to correspond with the impact-toughness, the latter being determined by the single-blow method. While such impact-toughness 40 drops quite rapidly with the addition of nickel, as will be seen, the curve indicating this property becomes more nearly horizontal at higher percentages of added metal. The tensile strength on the contrary increases 45 rapidly at first, then more slowly and finally begins to fall off, while the Brinell hardness beginning with an alloy containing a little over 1 per cent of nickel increases rapidly with the addition of further nickel through- 50 out the range shown on the diagram.

In order to secure a proper balance in respect to the characteristics in question, I prefer to employ between 5 per cent and 8 per cent of nickel, castings made from such resulting alloy having a specific gravity of 60 from 1.80 to 1.90; tensile strength from 18,000 to 19,000 per square inch; Brinell hardness from 45 to 50; and single-blow impact-toughness from 40 to 30.

As previously indicated, where it is desired to modify the characteristic of hardness and particularly the brittleness which is associated therewith in the case of the binary alloy under consideration, I have found that the addition of a small proportion 65 of aluminum, or of aluminum and zinc, is 70 advantageous. A satisfactory formula for a ternary alloy using my improved binary magnesium-nickel alloy as a base is as follows, viz, magnesium 90 per cent; nickel 6 75 per cent; and aluminum 4 per cent. Where in addition to aluminum zinc is added as an ingredient, the following formula has been found to give satisfactory results; magnesium 90 per cent; nickel 5 per cent; aluminum 3 per cent; and zinc 2 per cent. 80

Even when the amount of aluminum added is relatively larger than that of nickel, the characteristic effects of the latter ingredient are retained to a noticeable degree, 85 as for example in the following ternary alloy, viz; magnesium 90 per cent, aluminum 8 per cent, and nickel 2 per cent.

To make my improved alloy, a measured quantity of pure magnesium metal is first 90 melted in a suitable pot along with the proper amount of a flux that while heavier than such metal will have proper surface tension to promptly and effectively coat the metal. As an example of such a flux, approximately equal parts of anhydrous magnesium chloride and sodium chloride may 95 be employed and if the specific gravity of the resultant mixture proves inadequate to float the metal after it has been alloyed, a small amount of barium chloride may be 100 added. A relatively small portion of the molten magnesium metal is then taken up in a ladle and the whole or part of the nickel, depending upon the total percentage 105 thereof to be added to the batch, is first placed in such ladle and melted with the magnesium therein, thereby producing an alloy very high in nickel. In order to insure the interfusing of the nickel with the 110

magnesium, it is necessary that it be in finely divided form such as wire, or else it may be powdered before being added. The contents of the ladle are then gradually added 5 to the main body of molten magnesium with the result that the nickel will diffuse throughout the mass and not drop through into the body of flux in which the latter floats and so be lost. As soon as the introduction 10 of the nickel alloy has been effected, the whole mass is well puddled and the operation may then be regarded as complete and the molten alloy cast either into ingots or directly into the form of the mechanical 15 parts for which it is intended to be used.

Where either aluminum or zinc, or both, are to be added to the binary alloy in accordance with formulas such as hereinbefore set forth, the relatively small amount 20 of such additional metal or metals may be separately introduced in the same fashion as the nickel, or they may be at once added along with the latter in forming the preliminary alloy which is subsequently added to 25 the main body of the molten magnesium metal, resulting in the production of an alloy in which such magnesium is the predominant ingredient, while of the other ingredients the nickel is relatively the larger 30 in amount. In some cases, moreover, when more than one metal is to be added to the magnesium, such metals may be first combined together and added in the form of the resulting alloy, which may contain a relatively 35 low percentage of magnesium if desired.

For convenience in defining the relative proportions of the metals that enter into the alloy, the magnesium may be referred to as 40 present in predominant amount, meaning an amount on the order of 80 per cent or more of the total; while in referring to the presence of other constituents in substantial but relatively small amounts, it will be understood 45 that amounts are meant on the order of those specified in the formulas hereinbefore set forth, due regard being given to the fact that the total of such other ingredients will decrease as the amount of the predominant 50 constituent is increased.

Other modes of applying the principle of my invention may be employed instead of the one explained, change being made as regards the steps herein disclosed or the ingredients 55 employed in carrying out such steps, provided the steps or ingredients set forth in the following claims or the equivalent of such steps or ingredients be employed.

60 I therefore particularly point out and distinctly claim as my invention:—

1. As a new product, an alloy containing magnesium and nickel, wherein the magnesium largely predominates, said alloy having 65 a tensile strength in excess of 18,000

70 pounds per square inch, Brinell hardness approximately 45 and single-blow impact-toughness between 40 and 30.

2. As a new product, an alloy containing not less than eighty nor more than ninety-nine and one-half per cent of magnesium and not more than twenty nor less than one-half of one per cent of nickel, said alloy having a tensile strength in excess of 18,000 75 pounds per square inch, Brinell hardness approximately 45 and single-blow impact-toughness between 40 and 30. 75

3. As a new product, an alloy containing from ninety to ninety-four per cent of magnesium and from six to eight per cent of nickel, said alloy having a tensile strength in excess of 18,000 pounds per square inch, Brinell hardness approximately 45 and single-blow impact-toughness between 40 and 30. 80

4. As a new product, an alloy containing 85 magnesium, nickel and aluminum, wherein the magnesium largely predominates and the remaining constituents are present in substantial but relatively small amounts.

5. As a new product, an alloy containing magnesium, nickel and aluminum, wherein the magnesium largely predominates and the remaining constituents are present in substantial but relatively small amounts, the nickel being in excess of the 80 aluminum. 85

6. As a new product, an alloy containing magnesium, nickel, aluminum and zinc, wherein the magnesium largely predominates and the remaining constituents are present in substantial but relatively small amounts, the nickel being in excess of the aluminum and the amount of the latter being approximately the same as that of the 100 zinc. 100

7. As a new product, an alloy containing magnesium, nickel, aluminum and zinc, wherein the magnesium largely predominates and the remaining constituents are present in substantial but relatively small amounts, the nickel being in excess of the aluminum and the amount of the latter being slightly greater than that of the zinc. 110 105

8. As a new product, an alloy containing not less than eighty nor more than ninety-nine and one-half per cent of magnesium, not more than twenty nor less than one-half of one per cent of nickel, and aluminum in substantial but relatively small proportion. 115

9. As a new product, an alloy containing not less than eighty nor more than ninety-nine and one-half per cent of magnesium, not more than twenty nor less than one-half of one per cent of nickel, and aluminum and zinc in substantial but relatively small 120 proportions. 120

10. As a new product, an alloy containing approximately the indicated percentages of the following metals, viz:—magnesium ninety per cent, nickel five per cent, alu- 130

minimum three per cent and zinc two per cent.

11. The method of making a magnesium-nickel alloy, which consists in first inter-fusing the desired amount of nickel with a relatively small quantity of the total magnesium in such alloy, and then adding the resulting alloy to the remaining quantity of magnesium in molten state.

12. The method of making a magnesium-nickel alloy, wherein the magnesium largely

predominates, which consists in first inter-fusing the desired amount of nickel with a relatively small quantity of magnesium, whereby an alloy relatively high in nickel is produced, and then adding such resulting <sup>15</sup> alloy to the remaining quantity of magnesium.

Signed by me this 24th day of October, 1921.

JOHN A. GANN.